

## UNITED STATES PATENT OFFICE

2,149,314

## PYROTECHNIC COMPOSITION

George J. Schladt, Dover, N. J.

No Drawing. Application February 16, 1938,  
Serial No. 190,806

9 Claims. (Cl. 52—24)

(Granted under the act of March 3, 1883, as  
amended April 30, 1928; 370 O. G. 757)

The invention described herein may be manufactured and used by or for the Government for governmental purposes without the payment to me of any royalty thereon.

5 The subject of this invention is a pyrotechnic composition.

As disclosed in Patent No. 2,035,509 of March 31, 1936, a coating and binding agent of paraffin is used in an illuminating composition comprising 10 magnesium and nitrates of barium and strontium. Storage tests of this composition have shown that the paraffin tends to flow and either segregates or becomes absorbed by the paper containers. This results in loss of binding action and also in 15 loss of a protective coating for the magnesium so that as a consequence the efficiency of the composition is greatly reduced.

The purpose of this invention is to provide a coating and binding agent for a pyrotechnic composition which avoids the above enumerated disadvantages of paraffin and which will be satisfactory with respect to candle power, burning rate and stability.

The improved agent consists of a mixture of a 25 drying oil, such as linseed or tung oil, and a non-drying or semi-drying oil, such as castor oil or soya bean oil. When a drying oil alone is used the solidification process proceeds too rapidly resulting in shrinkage faults and cavities. When 30 a non-drying oil alone is used the solidification process proceeds too slowly resulting in unsatisfactory binding of the surfaces of the ingredients.

A composition having the following ingredients has given excellent results:

|                   | Percent |
|-------------------|---------|
| Barium nitrate    | 36-40   |
| Strontium nitrate | 6-8     |
| Magnesium, coated | 50-54   |
| Castor oil        | 1-4     |
| Linseed oil       |         |

The magnesium is preferably coated with linseed oil before being introduced into the composition to insure its protection against oxidation while providing a desirably high candlepower value and a suitable burning rate.

I claim.

1. A composition consisting of barium nitrate, strontium nitrate, magnesium coated with linseed oil, and a binding agent of one to four percent of a mixture of linseed oil and castor oil. 10

2. A composition consisting of barium nitrate, strontium nitrate, magnesium, and a binding agent of one to four percent of a mixture of linseed oil and castor oil.

3. A composition consisting of barium nitrate, strontium nitrate, magnesium coated with a drying oil, and a binding agent of one to four percent of a mixture of a drying oil and a non-drying oil.

4. A composition consisting of barium nitrate, strontium nitrate, magnesium, and a binding agent of one to four percent of a mixture of a drying oil and a non-drying oil.

5. A pyrotechnic composition including magnesium coated with linseed oil, and a binding agent consisting of a mixture of linseed oil and castor oil. 25

6. A pyrotechnic composition including magnesium coated with a drying oil, and a binding agent consisting of a mixture of a drying oil and 30 a non-drying oil.

7. A pyrotechnic composition including magnesium coated with a drying oil.

8. A pyrotechnic composition including a binding agent consisting of a mixture of linseed oil 35 and castor oil.

9. A pyrotechnic composition including a binding agent consisting of a mixture of a drying oil and a non-drying oil.

GEORGE J. SCHLADT. 40